

Patented Aug. 30, 1927.

## UNITED STATES PATENT OFFICE.

PHILIP W. DAVIS, OF CAMBRIDGE, MASSACHUSETTS.

## REFINING LEAD.

No Drawing.

Application filed January 11, 1926. Serial No. 80,672.

The present invention relates to an improvement in refining lead.

The object of the invention is to produce a very pure lead from lead alloys by a two-step process. In the first step the greater part of the alloy metals are removed, and in the second step the entire remainder, or substantially the entire remainder, of the alloy metals are removed, and a lead of high purity is secured. The invention consists in the method of refining lead herein-after described and particularly defined in the claims.

A specific embodiment of the present invention will be described. The product of smelting scrap storage battery plates carries from 3% to 5% of antimony. This lead antimony alloy is treated by melting it and pouring it into a cast iron vessel, and then introducing into the vessel a suitable quantity of pulverulent litharge. The temperature of the lead will be between approximately 600° C. and approximately 883° C. These temperatures are respectively the melting points of litharge carrying antimony and of pure litharge. The lead alloy and litharge will then be stirred by any suitable means, and the litharge and lead will be brought into intimate contact with each other in bodies of small masses, and the litharge will take up from the lead a large quantity of the antimony present. Thus, the lead by this low temperature method may be reduced, for example, from 3.62% antimony to .05% antimony at a temperature of 680° C.

This preliminarily refined lead still has an antimony content beyond that which is desired for some uses to which the metal lead is put, and in order to remove the remaining antimony, or substantially all of the remaining antimony, it is then subjected to a second step, which consists in mixing molten litharge with the molten lead containing this small percentage of antimony in a suitable furnace, and maintaining the temperature above the melting point of litharge.

While in the first step of the process it was not necessary that the litharge should be entirely free from antimony, in the second step it is preferred to use litharge which is substantially free from antimony, although good results may be obtained by the use of litharge containing a small amount of antimony, as it will retain such antimony and take up more antimony from the lead

alloy. The intimate mixture of the molten litharge with the molten lead containing the small residual amount of antimony in bodies of small dimensions and at temperatures above the melting point, 883° C., of litharge, is a rapid operation, which results in reducing the amount of antimony present in the lead alloy to an extremely small amount. Thus, a degree of purity of lead has repeatedly been secured which contained only .003% antimony. It has also been carried to such a degree of purity as to show only a trace of antimony.

It will be noted that the present invention contemplates a two-step method of removing antimony from lead, of which the first step is carried on at a low temperature, that is to say, a temperature below the melting point of pure litharge, and the second step is carried on at a high temperature, that is to say, at a temperature somewhat above the melting point of pure litharge. The first step removes a very large percentage of the antimony present, and the second step removes substantially all of the remaining antimony. The first step may be carried on at low temperatures and with an inexpensive plant and in large batches. The second step will be carried on at higher temperatures in a more expensive plant, but in smaller batches, because of the greater rapidity of the reaction.

While the present invention has been described in connection with a specific illustration of refining lead for the purpose of removing antimony, and while this is believed to be an important use of the process because of the large quantities of antimonial lead which are available from lead storage battery plates, and because of its availability in the refining of other leads containing antimony, still it is to be understood that the invention is not limited to this particular application, as the process may be employed for the removal of other metals from lead by oxidation by the use of litharge.

Having thus described the invention, what is claimed is:

1. The method of refining lead which consists in first exposing lead alloys in molten condition to the action of pulverulent litharge by causing the two materials to be exposed to each other in bodies of small dimensions and at temperatures between the melting point of litharge carrying the alloy metal and the melting point of pure litharge,

and second, subjecting the lead alloy product of the first step in molten condition to the action of molten litharge by causing the two materials to be exposed to each other in bodies of small dimensions at temperatures above the melting point of pure litharge.

2. The method of refining lead which consists in first mixing lead alloy in molten condition with pulverulent litharge at temperatures between the melting point of litharge carrying the alloy metal and the melting point of pure litharge, and second, in mixing the molten lead alloy product of the first step with molten litharge at temperatures above the melting point of pure litharge.

3. The method of refining lead antimony alloys which consists in first exposing the alloy in molten condition to the action of pulverulent litharge at temperatures between the melting point of litharge carrying antimony (approximately 600° C.) and the melting point of pure litharge (approximately 883° C.), and second, in mixing the molten alloy product of the first step with molten litharge at temperatures above the melting point of pure litharge (approximately 883° C.).

In witness whereof I have signed my name to this specification.

PHILIP W. DAVIS.